

(No Model.)

2 Sheets—Sheet 1.

A. F. OPPERMANN.

FILAMENT FOR INCANDESCENT ELECTRIC LAMPS.

No. 408,740.

Patented Aug. 13, 1889.



Fig. 1.



Fig. 3.



Fig. 2.



Fig. 4.

Witnesses.

Cly Hawley  
Geo. R. Parker.

Inventor.

Adolf F. Oppermann  
By George P. Burton  
Attorney.

(No Model.)

2 Sheets—Sheet 2.

A. F. OPPERMANN.

FILAMENT FOR INCANDESCENT ELECTRIC LAMPS.

No. 408,740.

Patented Aug. 13, 1889.



Fig. 5.

Witnesses.

C. G. Hawley.

Geo. R. Parker.

Inventor.

Adolf F. Oppermann.

H. C. George & Beaton  
Attorney.

# UNITED STATES PATENT OFFICE.

ADOLF F. OPPERMANN, OF CHICAGO, ILLINOIS.

## FILAMENT FOR INCANDESCENT ELECTRIC LAMPS.

SPECIFICATION forming part of Letters Patent No. 408,740, dated August 13, 1889.

Application filed April 11, 1889. Serial No. 306,848. (No model.)

*To all whom it may concern:*

Be it known that I, ADOLF F. OPPERMANN, a subject of the Queen of Great Britain, residing at Chicago, in the county of Cook and State of Illinois, have invented a certain new and useful Improvement in Incandescent Electric Lamps, of which the following is a full, clear, concise, and exact description, reference being had to the accompanying drawings, forming a part of this specification.

My invention relates to the manufacture of incandescent lamps, and more especially to the filament; and its objects are, first, to increase the life of the filament; second, to prevent its becoming warped or bent, and, third, to secure a battery-connection between the leading-in wires and the ends of the filament. Heretofore the filament has been made from different kinds of vegetable fiber—strips of paper, cotton yarn, bamboo, and grasses of different varieties having been used in their manufacture. The filaments, after being carbonized, have been subjected to an electric current while surrounded by hydrocarbon gas. The filament, being thus surrounded and heated, is re-enforced by a coating of carbon taken up from the gas. When cotton yarn has been used, the filaments often become distorted, owing to the tendency of the fiber to untwist, even after being carbonized. Cements of various kinds have been used for mounting the filaments upon the ends of the platinum wires leading in through the globe. India-ink mixed with stove-polish has sometimes been used for this purpose.

My invention consists in subjecting the cotton thread to a high degree of pressure, so as to crush the fiber before it is carbonized, so as to avoid the distortion of the filament, heretofore resulting from the tendency of the fiber to untwist.

My invention consists, also, in subjecting the carbonized filament to the action of an alternating current while the filament is surrounded by hydrocarbon gas, so as to make the coating or deposit thickest at the upper portion or curve of the filament.

I preferably make use of a mixture of india-ink and platinum-black as a cement for mounting the filament upon the leading-in wires, this cement having been found by me

more satisfactory than other cements now in use.

My invention is illustrated in the accompanying drawings, in which—

Fig. 1 is a side elevation of a machine adapted to crush the fiber of the cotton yarn. Fig. 2 is a side elevation of a lamp provided with a filament embodying my invention. Figs. 3 and 4 are detail views of the filament. Fig. 5 is a sectional view of a tank containing gasoline and illuminating-gas, a filament being inserted therein for the purpose of receiving the carbon coating.

Referring now to Fig. 1, the rollers *a* should be smooth and fitted closely together, like jewelers' rolls used for flattening sheet metal. The end of the cotton yard or thread is placed between these rolls, and the crank being turned the thread is drawn through and compressed to such an extent as to prevent any tendency of the fiber to untwist. The thread being thus compressed, I next cut it into the lengths required, after which the separate pieces are carbonized. The next step in the manufacture is to coat these filaments with a deposit derived from the hydrocarbon, this coating being made thicker at the curved or upper portion of each filament. In order that such increased thickness may be obtained, I send current in alternations through each filament while surrounded by the hydrocarbon. I also preferably place the curved portion in an atmosphere of denser gas than that which surrounds the legs of the filament. Thus, as shown more clearly in Figs. 2 and 3, the curved portion *b* of the filament has received a thicker coating than the legs *c*. This is caused by the alternating current heating the curved portion to a greater extent than the legs or sides are heated, and also on account of subjecting the curved portion to a denser atmosphere of gas.

The filament is secured to the platinum leading-in wires *d* by cement *e*, consisting of a mixture of india-ink and platinum-black, a small proportion of the platinum-black being sufficient. I preferably use one part of platinum-black to twenty parts of india-ink.

The preferable manner of coating the filament is illustrated in Fig. 5. A vessel *f* containing gasoline of sufficient depth to cover

the filament when inserted therein is surrounded by the gas-chamber *g*, a small opening being provided, preferably in the top of the gas-chamber, through which the filament 5 may be inserted. The holder *h* is provided with clamps *i*, and the ends of the filament are held, as shown, by these clamps. The holder contains wires connected with a suitable source of alternating current, these wires 10 being connected with the metal springs of the clamps, so that when the filament is inserted therein said filament will be included in the circuit over which the current is being sent in alternations. This current should be 15 of sufficient strength to heat the filament to incandescence, and, as is well understood, the upper or central portion of the filament will be heated more than the sides.

The filaments are placed upon the holder 20 one after another, each being subjected to the action of the alternating current while immersed in the gasoline and, preferably, for a short time—say four or five seconds—while the curved portion is above the surface of the 25 gasoline and surrounded by the dense hydrocarbon gas, while the legs or sides are covered by the gasoline. The upper portion, which is surrounded by the gas under these conditions, will be heated to a much higher 30 temperature than the portion which is immersed in the gasoline. I preferably use at the same time the alternating current and also suitable means for bringing the gas against the upper portion only of the filament. A 35 continuous current would cause a thicker deposit upon the curved portion if the gas about said portion were more dense than about the sides of the filament; but the same effect would be produced if the gas were entirely 40 prevented from coming in contact with the sides while the upper portion was surrounded. The alternating current, however, in itself causes a thicker deposit at the curved portion of the filament—that is to say, at the central 45 portion of the resistance thereof, though the gas surrounding the entire filament should be of the same density.

Lamps provided with filaments which have received a thicker coating at the upper or 50 curved portion thereof, as hereinbefore described, and which are secured to the leading-in wires by a cement of india-ink and platinum-black are more durable, especially in

alternating systems, than any lamps heretofore in use, the tendency of the filament to 55 break at the central portion of its resistance being compensated for and overcome by the greater thickness of the coating.

Having thus described my invention, I claim as new and desire to secure by Letters Patent— 60

1. The method of manufacturing filaments for incandescent lamps, which consists in crushing the twisted fiber of the filament, carbonizing the same, and then subjecting the filament thus carbonized to the action of an 65 alternating current while surrounded by hydrocarbon gas, substantially as and for the purpose specified.

2. The process of manufacturing filaments for incandescent lamps, which consists in 70 crushing the twisted fiber before it is carbonized, then carbonizing the filament and subjecting the same to an alternating current while surrounded by hydrocarbon gas, the 75 gas being denser at the upper or curved portion of the filament, substantially as and for the purpose specified.

3. In the manufacture of a filament for an incandescent lamp, the process consisting of 80 subjecting the carbonized filament to the action of an alternating current while surrounded by hydrocarbon gas, the exposure to the hydrocarbon gas at the curved portion thereof or central portion of the resistance thereof being continued for a greater time 85 than the exposure of the other portions thereof, whereby the coating is made thicker at the said central or curved portion thereof, substantially as and for the purpose specified.

4. The method of manufacturing filaments 90 for incandescent lamps, which consists in crushing the twisted fiber of the filament, carbonizing the same, and then subjecting the filament thus carbonized to the action of an electric current while surrounded by hydrocarbon gas, the curved portion or center 95 of resistance of the filament being exposed longer to the gas than the other portions of the filament.

In witness whereof I hereunto subscribe my 100 name this 8th day of April, A. D. 1889.

ADOLF F. OPPERMANN.

Witnesses:

GEORGE P. BARTON,  
ELLA EDLER.